# EUROPEAN PATENT SPECIFICATION

(11) **EP 0 830 479 B1**
(45) Date of publication and mention of the grant of the patent: **07.03.2007**
(21) Application number: 96901357.2
(22) Date of filing: 25.01.1996
(51) Int. Cl.: D21H 21/16, D21H 17/17

(54) **A METHOD FOR INCREASING THE HYDROPHOBICITY OF PRINTING PAPERS**
VERFAHREN ZUR ERHÖHUNG DER WASSERFESTIGKEIT VON DRUCKPAPIEREN
PROCEDE D'AMELIORATION DE L'HYDROPHOBICITE DE PAPIERS D'IMPRESSION

(30) Priority: 25.01.1995 FI 950326
(43) Date of publication of application: 25.03.1998
(62) Divisional of application: 05002881.0
(73) Proprietor: Ciba Specialty Chemicals Holding Inc., 4057 Basel (CH)
(72) Inventor: ZETTER, Claes, FIN-20810 Turku (FI); MALMSTRÖM, Olof, FIN-20880 Turku (FI); NURMINEN, Markku, FIN-21120 Raisio (FI)
(74) Representative: Lalli, Esko
(86) International application number: PCT/FI1996/000051
(87) International publication number: WO 1996/023105

(56) References cited:
- EP-A- 0 220 941
- EP-A- 0 610 895
- WO-A-94/01619
- WO-A-94/05855
- DE-A- 3 104 576
- US-A- 5 145 522

## Description

The present invention relates to a method of improving the hydrophobicity of printing papers by means of internal sizing of the paper. A particular object of the invention is to improve the hydrophobicity of paper by means of using a ketene dimer compound as a hydrophobic sizing agent. The purpose of improving the hydrophobicity is to impart the paper web a degree of sizing that makes the paper compatible with ink-jet printing.

The resistance properties of paper to wetting and penetration are conventionally enhanced in papermaking by means of internal sizing, where during the paper making process compounds are added into the paper pulp which increase the hydrophobicity of the paper fibers.

Printing papers, which are chiefly used as office paper in various types of copiers, printers and printing machines, are expected to exhibit high brightness among other properties, as well as acceptable permanence in archive document use. The brightness and archiving permanence properties can be affected through the type of filler used for the paper. One filler compatible with the above-described requirements is precipitated calcium carbonate (PCC). However, a problem is involved in the use of this filler, because it requires a neutral or alkaline environment for a proper functioning. Such a process condition excludes the use of conventional hydrophobic sizing of paper by means of the rosin-alum system. As known in the art, this drawback is overcome by the use of hydrophobic sizes based on ketene dimer compounds such as alkyl, alkenyl, aryl and alkaryl ketene dimer sizes.

Such sizes are, however, hampered by other problems particularly in paper grades intended for office printing use that have to be compatible with different printer types. Namely, besides a application in ink-jet printing, the same paper grade should do as copier paper, laser printing paper, etc. When optimized for the above-mentioned ink-jet use, the base paper must be sized with such great amounts of ketene dimer combination sizes that ultimately the size causes problems in the alternative printer types. In practice, the degree of sizing may amount to, e.g., 0.1 - 0.2 % of fiber dry weight in the web.

Over time, ketene dimer compounds have been found problematic as a sizing agent due to their migration tendency in the finished paper. Owing to such migration, the content of the ketene dimer compound is enriched in the outer layers of the sheet. Migration is made possible by the fact that the curing reactions of ketene dimer compounds are so slow that the added agents lose their migration capability not earlier than after a few days from the finishing of the sheet.

A disadvantageous effect of ketene dimer compound enrichment is easier slippage of the sheet surface, i.e., decrease of surface frictional resistance. Reduced friction is harmful particularly in printing and copier paper grades, because the lowered threshold of slippage causes paper handling problems in printing or copying machines whose paper transfer elements fail to provide their intended function on slippery paper grades.

Also the above-mentioned filler, namely, the precipitated calcium carbonate causes indirectly easier slippage of the sheet. This is because this filler has been found to disturb the hydrophobic sizing process, whereby greater amounts of size must be used per unit weight of fiber in comparison to the use of another type of filler.

On the other hand, it has been found that ketene dimer based sizing fails to bond completely on the fiber during sheet formation, whereby a fraction of the sizing agent remains circulating in the system and of this fraction a portion bonds later on the fiber. When circulating in the system, the sizing compound is subjected to the hydrolyzing effect of water resulting in a partial decomposition of the sizing compound into corresponding ketones. Also a fraction of the size retained in the base web will remain unbonded to the fiber, whereby the size may undergo hydrolyzation by the moisture contained in the web. These phenomena are harmful particularly in copier use, where the sheet is subjected to heating in the copying machine, whereby the decomposition of unbonded size and its migration, along with the moisture released from the sheet, to the surface of the sheet are accelerated. Resultingly, the machine parts of the copier may become contaminated and the copying result deteriorated. To eliminate these risks, determination of residual ketone content in paper grades intended for copier use has been instigated.

Blixt, T. R. , "Chalk - A Calcium Carbonate for the High-Filled Sheet", Paper presented at 1992 Papermakers Conference 5-8 April 1992, Nashville, TN, USA, Book 2, pp 515-520, Tappi Press 1992 discloses a paper making process using PCC as filler. In the process alkyl ketene dimer is added to the machine chest at a rate of 0.5 to 2 kg/ton and starch is added to the thick stock at a rate of 5 kg/ton.

EP-A1-0 220 941 discloses a paper sizing composition for internal sizing of paper, including ketene dimers as sizing ingredients in a water dispersable encapsulation agent, such as starch in an amount of 25 to 100% by weight of the ketene dimer present in the dispersion.

The publication US-Al-5,145,522 discloses internal sizing of papers in neutral or alkaline conditions, wherein the ketene dimer size is stabilized by a polymeric aluminium compound used together with a dispersing agent, such as cationic starch the starch being used in an amount of 0.5 to 100 % by weight against the ketene dimer used.

EP-A1-0 610 893 discloses a surface size composition for paper. The composition comprises 50 - 99.9 wt% fully hydrolyzed PVOH and 0.1 - 50 wt% ketene dimer compound (solid/solids).

DE-A1-31 04 576 discloses compositions for internal sizing of paper using AKD and ASA, and a cationic galactomannan as protective colloid for these sizing agents, in the amounts of 0.1 to 1.5 times the reactive sizing agent.

According to the present invention, an essential improvement has now been achieved to overcome the above-described problem by virtue of a method of improving the ink-jet printability of printing paper manufactured using precipitated calcium carbonate as filler, by adding prior to web formation to the pulp slurry a ketene dimer compound, whereby a sizing dispersion is used that contains at least the ketone dimer compound as a hydrophobic sizing agent in an amount of 0.1-0.2 % of fiber dry weight and further contains water-soluble colloïdal polymer, and wherein the amount of the water-soluble colloidal polymer is at least 100 % by weight of the hydrophobic sizing agent.

Herein, it has firstly been noted that ketene dimer compound used as the hydrophobic sizing agent is better bonded to the fiber, and, secondly, that the precipitated calcium carbonate used as the filler has no essential disturbing effect on the sizing process. Owing to the latter fact, less is needed, whereby said smaller amount of the hydrophobic sizing agent can be retained close to the fiber in an improved manner until the curing of the hydrophobic sizing agent has proceeded to a level preventing migration. Additionally, it was found that the invention offered improved.ink penetration properties with respect to the water penetration. This effect is of extremely high importance to the quality of ink-jet printing that is becoming ever more widely used.

The invention has furthermore been found applicable in cases where the ketene dimer compound employed as a hydrophobic sizing agent in the sizing of paper is complemented with other conventional hydrophobic sizing agents such as alkylated succinic anhydride and/or rosin.

Particular embodiments of the invention are set out in the dependent claims.

The invention is next explained with the help of the following examples elucidating the function of the invention in its different embodiments.

### Example 1

A pilot-scale test run was carried out, in which internal sizing was performed for a finepaper grade with added precipitated calcium carbonate (PCC) as the filler. The filler (tradename Albacar LO) was used at 22 % level by fiber dry weight. The fiber in the base web was 75 % birch fiber beaten to 23 SR° freeness and the fiber slurry was adjusted to pH 7. The rest, 25 %, of the fiber was pine fiber equally beaten to 23 SR° freeness and fiber slurry also adjusted to pH 7, Raisamyl 135 was added to the pulp as stock starch at 5 kg/ton addition rate. The basis weight of the produced paper web was 80 g/m². The paper machine was run at 60 m/min resulting in a production rate of 4.08 kg/min. The retention agent used in the process was BMA 590 (colloidal sodium silicate) at an addition rate of 300 g/ton pulp. The paper web was also surface sized using Raisamyl 406 LO starch at 6 % solids addition level. The hydrophobic compound used as a sizing agent was alkyl ketene dimer (AKD).

The test runs were performed using the different formulations of hydrophobic size listed below for internal sizing:
1. Conventional AKD sizing with Raisafob 940, in which the amount of starch protective colloid addition was not more than 20 % by weight of sizing agent.
2. AKD sizing, amount of starch protective colloid addition 50 % by weight of sizing agent.
3. AKD sizing, amount of starch protective colloid addition 100 % by weight of sizing agent.
4. AKD sizing, amount of starch protective colloid addition 150 % by weight of sizing agent.
5. AKD sizing, amount of starch protective colloid addition 200 % by weight of sizing agent.
6. AKD sizing, amount of starch protective colloid addition 250 % by weight of sizing agent.
7. AKD sizing, amount of starch protective colloid addition 300 % by weight of sizing agent.
8. AKD sizing, amount of protective colloid addition using PEI (polyimin KK)* in an amount of 200 % by weight of sizing agent.
Notes: *) polyethylene imine

The tests were run using two levels of sizing agent, namely, adding the sizing agent (AKD) at 0.1 % and 0.2 % levels by fiber dry weight.
The starch used as the protective colloid component was Raisamyl 150 EH which is a degraded special starch grade.

The degree of sizing in the manufactured papers were tested by measuring the water absorbance of the paper sheets in the Cobb₆₀ test from the sheet surface, while the ink penetration of the sheets was measured using the Schröder test. Also the brightness of test sheets was measured.

The test runs gave the following results:

| Test no./ | Cobb₆₀ test [g/m²] | | Schröder test (100->90%, s) | | Brightness |
|---|---|---|---|---|---|
| Amount of size | 0.1 % | 0.2 % | 0.1 % | 0.2% | [%] |
| 1 | 78.2 | 28.3 | 0 | 10 | 92.7 |
| 2 | 76.3 | 28.1 | 1 | 11 | 92.6 |
| 3 | 41.5 | 26.6 | 2 | 15 | 92.7 |
| 4 | 29.3 | 20.2 | 5 | 135 | 92.8 |
| 5 | 25.0 | 18.4 | 18 | 248 | 93.0 |
| 6 | 24.8 | 18.3 | 20 | 253 | 92.9 |
| 7 | 24.7 | 18.2 | 21 | 255 | 93.0 |
| 8 | 28.8 | 18.1 | 21 | 262 | 91.1 |

From the above results it can be seen that, at an addition rate of the sizing agent of 0.1 % by fiber dry weight, a sufficient addition rate of the protective colloid component is at approx. 200 % level by hydrophobic sizing agent solids weight, whereby this combination provides such a Cobb₆₀ value of less than 25 g/m² that conventionally is considered to represent a sufficient level of sizing. For the larger, 0.2 wt.%, addition rate of the sizing agent, the corresponding water repellency value is attained using an addition rate of the protective colloid component as low as 100 % of the hydrophobic sizing agent solids weight. Also polyethylene imine (PEI) was found (test run no. 8) to act as a protective colloid component at the same addition rate (200 %), however, with the penalty that paper brightness is adversely affected particularly in grades manufactured using optical brighteners. The ink penetration property of the paper web is improved significantly up to 200 % addition rate of the protective colloid component, whereafter this property at higher addition rates stays approximately at the same level as when using PEI.

### Example 2

A production-scale test run was performed on a finepaper machine by making paper at 78 g/m² basis weight. The paper was manufactured using pulp comprised in 60/40 ratio of birch to pine fiber. The amount of filler added to the base web was at 22 % level by fiber dry weight, whereby 70 % of the filler was precipitated calcium carbonate (PCC, Albacar LO) and 30 % of ground CaCO₃. The retention system was formed by corn starch and an anionic component (Compozil).

The AKD sizing was applied using two different formulations:
1. Raisafob 940, conventional AKD sizing, amount of protective colloid component not more than 20 % of sizing material dry weight.
2. Raisafob 500, AKD sizing using starch as the protective colloid component with an amount increased to 200 % of size dry weight. The starch added as the protective colloid component was Raisamyl 150 EH.

The test runs were carried out using AKD sizing at 0.12 % level by fiber dry weight. Tests were performed in multiple series using both of the above sizing formulations in identical conditions to eliminate random error from the results. The test data is listed in the table below:

| Test run no. | AKD type | Cobb₆₀ | | Schröder test (100->91%, s) | Coefficient of friction | | Ink-jet, black-and-white | | | Ink-jet, color | | | |
|---|---|---|---|---|---|---|---|---|---|---|---|---|---|
| | | felt side | wire side | felt side | static | kinetic | black density (100%) | ink drying time [s] | wicking mean | ink drying time [s] | wicking mean | color-to-color bleeding | black density (100%) |
| 77 | RF940 | 21.7 | 22.2 | 59 | 0.79 | 0.54 | 1.60 | 9 | 4 | 19 | 10 | 8 | 1.08 |
| 79 | RF940 | 20.7 | 21.5 | 49 | 0.67 | 0.50 | 1.64 | 11 | 4 | 20 | 10 | 8 | 0.98 |
| 81 | RF940 | 21.2 | 20.7 | 54 | 0.77 | 0.54 | 1.64 | 9 | 6 | 18 | 10 | 8 | 0.97 |
| 84 | RF940 | 20.4 | 20.6 | 78 | 0.75 | 0.58 | 1.76 | 12 | 4 | 15 | 10 | 8 | 1.03 |
| 87 | RF500 | 19.9 | 19.8 | 205 | 0.76 | 0.53 | 1.91 | 22 | 2 | 109 | 10 | 8 | 1.38 |
| 89 | RF500 | 19.3 | 19.0 | 181 | 0.75 | 0.53 | 1.93 | 14 | 2 | 144 | 10 | 8 | 1.38 |
| 91 | RF500 | 19.4 | 19.2 | 209 | 0.82 | 0.57 | 1.94 | 21 | 2 | 154 | 10 | 8 | 1.42 |
| 93 | RF500 | 19.4 | 19.4 | 203 | 0.81 | 0.57 | 1.90 | 19 | 2 | 157 | 10 | 8 | 1.46 |
| 95 | RF500 | 19.5 | 18.9 | 277 | 0.78 | 0.60 | 1.96 | 24 | 2 | 172 | 10 | 8 | 1.51 |

As is evident from the above results, sizing properties are clearly improved by the use of RF 500 and the coefficient of friction is simultaneously retained at the same level or even improved. The ink-jet printing tests indicate that the use of RF 500 gives positively improved black-and-white printing results over conventional sizing, and simultaneously, the ink-jet color printing test remains unchanged, which indicates that the level of sizing herein is overproportioned for ink-jet color printing.

### Example 3

A production-scale test run was carried out in which the following sizing formulations were compared:

| | | |
|---|---|---|
| 1. | Raisafob 940 | AKD sizing, amount of starch protective colloid addition not more than 20 % by weight of sizing agent. |
| 2. | Raisafob 500 | AKD sizing, amount of starch protective colloid addition 200 % by weight of sizing agent. |

The paper made herein was a office paper grade intended for multipurpose use. The production target values for the paper grade were set as follows : residual ketone content less than 0.4 mg/g (for copier use), black density greater than 1.2 in B/W printing on ink-jet printers and combination black density greater than 0.75 in multicolor printing.

Test run conditions:
- Paper grade:: Office paper (multipurpose)
- Basis weight:: 80 g/m²
- Base web composition:: 70% birch fiber at 23 °SR freeness
30% pine fiber at 23 °SR freeness
- Filler:: Precipitated calcium carbonate (PCC)
- Retentionsystem:: Two-component formulation (polymer + bentonite)
- Surface sizing:: Raisamyl 408 starch + 1.5 kg styrene acrylate polymer/ton pulp solids
- Paper machine speed:: 980 m/min
- AKD addition rate:: 1 kg AKD/ton pulp solids, or alternatively, 1.4 kg AKD/ton pulp solids

### Test results:

| Sizing agent | Addition rate [kg/ton] | Cobb₆₀, [g/m²] | Ink penetration HST 80 [%, s] | Residual ketone [mg/g] | Black density, B/W printing, felt side | Black density, comp. color printing, felt side |
|---|---|---|---|---|---|---|
| RF940 | 1 | 25 | 80 | 0.41 | 1.02 | 0.64 |
| RF940 | 1.4 | 23 | 153 | 0.68 | 1.22 | 0.82 |
| RF500 | 1.4 | 21 | 238 | 0.27 | 1.38 | 0.90 |

As is evident from the above results, the sizing properties are clearly improved by the use of RF 500. Additionally, the residual ketone content remains below the set target value. Also the density target values set for ink-jet printing are exceeded. By contrast, using the RF 940 sizing formulation with a low protective colloid content it is not possible to meet the upper limit set for the residual ketone content. Hence, the paper made in this process is not suited for the intended copier use. If the size addition rate is reduced to a level of 1 kg/ton pulp solids, the RF 940 sizing formulation may marginally meet the level set for the maximum allowable residual ketone content, however, with the penalty of not meeting required ink penetration criteria.

The invention has further been found suitable for use in such paper sizing applications in which a fraction of the hydrophobic sizing agent is composed, besides of AKD, additionally of another sizing agent suited for improvement of water repellency such as alkenyl succinic anhydride (ASA). However, as ASA sizing formulations do not offer hydrophobic properties as effective as those of AKD sizing formulations, they must be used in larger amounts to achieve comparable ink-jet printability qualities. Due to the staining problems caused by the required large addition rates of ASA sizing in papermaking, this sizing approach appears less favored. However, because the use of an ASA sizing formulation in the present application would give a low residual ketone content in the finished sized paper, which is a definite benefit when using the paper in copiers. The well-known problematic properties of this sizing agent require that the sizing furnish be prepared in the immediate vicinity of the.papermaking process. In the following example, the behavior of this sizing formulation type is described.

### Example 4

A production-scale test run was carried out to compare the behavior of the following sizing formulations:

| | | |
|---|---|---|
| 1. | Raisafob 500 | AKD sizing, amount of starch protective colloid addition 200 % by weight of the ketene dimer. |
| 2. | Raisafob MF | ASA sizing, dispersed in stock starch Raisamyl 135 in an ASA/starch ratio of 1:2. |
| 3. | Raisafob 500 + Raisafob MF | AKD sizing plus Raisafob MF, added separately. |
| 4. | New sizing | AKD/Raisafob 500 type sizing formulation dispersion + ASA dispersed therein in AKD/ASA ratio of 50/50. |

The paper made herein was a office paper grade intended for multipurpose use. The production target values for the paper grade were set as follows: ketene content less than 0.4 mg/g (for copier use), black density greater than 1.2 in B/W printing on ink-jet printers and combination black density greater than 0.75 in multicolor printing.

Test run conditions:
- Paper grade:: Office paper (multipurpose)
- Basis weight:: 80 g/m²
- Base web composition:: 70 % birch fiber at 23 SR° freeness
30 % pine fiber at 23 SR° freeness
- Filler:: Precipitated calcium carbonate (PCC) at 20 % level by fiber dry weight
- Retention system:: Two-component formulation (polymer + bentonite)
- Surface sizing:: Raisamyl 408 starch + 1.5 kg styrene acrylate polymer/ton pulp solids
- Paper machine speed:: 980 m/min
- AKD addition rate:: 1.4 kg/ton (as AKD, RF500 pulp solids)
- ASA addition rate:: 1.4 kg/ton (RF MF)
- AKD/ASA addition rate:: 0.7 kg + 0.7 kg/ton (RF500 and RF MF, using separate additions)
- New sizing formulation:: 0.7 kg + 0.7 kg/ton (ASA dispersed in RF500 product)

### Test results:

| Sizing agent | Addition rate [kg/ton] | Cobb₆₀ [g/m²] | Ink penetration HST 80 [%,s] | Residual ketone [mg/g] | Black density, B/W printing, felt side | Black density, comp. color printing, felt side |
|---|---|---|---|---|---|---|
| RF500 | 1.4 | 22 | 24 | 0.29 | 1.32 | 1.06 |
| RF MF | 1.4 | 23 | 122 | 0 | 1.14 | 0.58 |
| RF500 +RF MF | 0.7+0.7 | 22 | 173 | 0.15 | 1.18 | 0.78 |
| New formulation | 0.7+07 | 21 | 208 | 0.15 | 1.21 | 0.86 |

As is evident from the above results, the requirements set for the compatibility of the manufactured paper with ink-jet printability are not met using ASA sizing alone. Admittedly, the paper exhibits zero residual ketone content. The novel type of combination sizing formulation is capable of meeting the requirements set for both copier and ink-jet printing use. The results also show the effect of the hydrolysis of ASA on the sizing efficiency when the ASA is dispersed in warm stock starch and then added separately. With regard to ink-jet printing, also herein the novel sizing formulation gives better density values than those achieved using ASA alone.

In a similar fashion as combining with ASA sizing, the AKD dispersion based on Raisafob 500 may be combined with rosin sizing. In general, rosin imparts good friction properties and does not make the paper slippery as typically is the case using AKD sizing alone.

## Claims

1. A method of improving the ink-jet printability of printing paper manufactured using precipitated calcium carbonate as filler, by adding prior to web formation to the pulp slurry a ketene dimer compound, **characterized in that** a sizing dispersion is used that contains at least the ketene dimer compound as a hydrophobic sizing agent in an amount of 0.1-0.2 % of fiber dry weight and further contains water-soluble colloidal polymer, and wherein the amount of the water-soluble colloidal polymer is at least 100 % by weight of the hydrophobic sizing agent.

2. A method as defined in claim 1, **characterized in that** a sizing dispersion is used in which the amount of the colloidal polymer is in the range of approx. 150 - 250 % by weight of the hydrophobic sizing agent.

3. A method as defined in claim 1, **characterized in that** a sizing dispersion is used containing at least one further sizing agent selected from the group consisting of alkenyl succinic anhydride and rosin.

4. A method as defined in any of claims 1 to 3, **characterized in that in that** said water-soluble colloidal polymer is selected from the group of compounds comprising: starches, carboxy methyl cellulose, ethyl cellulose, polyacryl amides, polyethylene imines, polyesters, polyethers, polyamides, polyvinyl alcohols, gelatine, tristearate, gum arabic, sugars or mixture thereof.

5. A method as defined in claim 4, **characterized in that** said water-soluble colloidal polymer is an amphoteric low-viscosity starch.

6. A method as defined in claim 3, **characterized in that** the further size component is an alkenyl succinic anhydride in an amount of 20 - 70%, advantageously 30 - 50 %, by weight of the ketene dimer.

7. A method as defined in claim 3, **characterized in that** the further size component is fortified rosin.

8. A method as defined in claim 3 or 7, **characterized in that** the further size component is rosin in an amount of approx. 20 - 50 % by weight of the ketene dimer compound.

9. A method as defined in any of claims 1 to 8, **characterized in that** the sizing dispersion further contains a surface-active compound, a biocidal agent and/or a pH-controlling agent.

10. A method as denned in claim 7 or 8, **characterized in that** the sizing dispersion contains aluminium sulphate at 2 - 15 % by weight of said colloidal polymer.

11. A method as defined in any of claims1 to 10, **characterized in that** said ketene dimer compound is selected from the group of alkyl, alkenyl, aryl and alkaryl ketene dimers.

12. A method as defined in any of claims 1 to 11, **characterized in that** the content of said hydrophobic sizing agent in the sizing dispersion is approx. 1-15 wt.%, advantageously 6-15 wt.%.

## Patentansprüche

1. Verfahren zur Verbesserung der Tintenstrahldruckfähigkeit von Druckerpapier, hergestellt unter Verwendung von ausgefälltem Calciumcarbonat als Füllstoff, indem vor der Bahnbildung eine Ketendimerverbindung zu der Fasermasse zugegeben wird, **dadurch gekennzeichnet, daß** eine Leimdispersion verwendet wird, die mindestens die Ketendimerverbindung als einen hydrophoben Leim in einer Menge von 0,1 bis 0,2 % des Fasertrockengewichtes enthält und außerdem wasserlösliches kolloides Polymer enthält, und wobei die Menge des wasserlöslichen kolloiden Polymers mindestens 100 Gew.-% des hydrophoben Leims beträgt.

2. Verfahren nach Anspruch 1, **dadurch gekennzeichnet, daß** eine Leimdispersion verwendet wird, in der die Menge des kolloiden Polymers im Bereich von ungefähr 150 bis 250 Gew.-% des hydrophoben Leims liegt.

3. Verfahren nach Anspruch 1, **dadurch gekennzeichnet, daß** eine Leimdispersion verwendet wird, die mindestens einen weiteren Leim enthält, ausgewählt aus der Gruppe, bestehend aus Alkenylbernsteinsäureanhydrid und Terpentinharz.

4. Verfahren nach einem der Ansprüche 1 bis 3, **dadurch gekennzeichnet, daß** das wasserlösliche kolloide Polymer aus der Gruppe aus Verbindungen ausgewählt ist, umfassend Stärke, Carboxymethylcellulose, Ethylcellulose, Polyacrylamide, Polyethylenimine, Polyester, Polyether, Polyamide, Polyvinylalkohole, Gelatine, Tristearat, Gummi arabicum, Zucker oder Gemische davon.

5. Verfahren nach Anspruch 4, **dadurch gekennzeichnet, daß** das wasserlösliche kolloide Polymer eine amphotere Stärke mit niedriger Viskosität ist.

6. Verfahren nach Anspruch 3, **dadurch gekennzeichnet, daß** die weitere Leimkomponente ein Alkenylbemsteinsäureanhydrid in einer Menge von 20 bis 70 Gew.-%, vorteilhafterweise 30 bis 50 Gew.-% des Ketendimers ist.

7. Verfahren nach Anspruch 3, **dadurch gekennzeichnet, daß** die weitere Leimkomponente verstärktes Terpentinharz ist.

8. Verfahren nach Anspruch 3 oder 7, **dadurch gekennzeichnet, daß** die weitere Leimkomponente Terpentinharz in einer Menge von ungefähr 20 bis 50 Gew.-% der Ketendimerverbindung ist.

9. Verfahren nach einem der Ansprüche 1 bis 8, **dadurch gekennzeichnet, daß** die Leimdispersion außerdem eine oberflächenaktive Verbindung, ein biozides Mittel und/oder einen pH-Regler enthält.

10. Verfahren nach Anspruch 7 oder 8, **dadurch gekennzeichnet, daß** die Leimdispersion Aluminiumsulfat bei 2 bis 15 Gew.-% des kolloiden Polymers enthält.

11. Verfahren nach einem der Ansprüche 1 bis 10, **dadurch gekennzeichnet, daß** die Ketendimerverbindung aus der Gruppe aus Alkyl-, Alkenyl-, Aryl- und Alkarylketendimeren ausgewählt ist.

12. Verfahren nach einem der Ansprüche 1 bis 11, **dadurch gekennzeichnet, daß** der Gehalt des hydrophoben Leims in der Leimdispersion ungefähr 1 bis 15 Gew.-%, vorteilhafterweise 6 bis 1 Gew.-% beträgt.

## Revendications

1. Procédé d'amélioration de l'imprimabilité par jet d'encre de papier d'impression fabriqué en utilisant du carbonate de calcium précipité en tant que charge, en ajoutant avant la formation de la bande un composé dimère de cétène à la suspension de pâte à papier, **caractérisé en ce qu'**une dispersion d'encollage est utilisée, qui contient au moins le composé dimère de cétène en tant qu'agent d'encollage hydrophobe, dans une quantité de 0,1 à 0,2% du poids sec de fibre, et qui contient en outre un polymère colloïdal hydrosoluble, et dans lequel la quantité de polymère colloïdal hydrosoluble est d'au moins 100% en poids de l'agent d'encollage hydrophobe.

2. Procédé selon la revendication 1,
**caractérisé en ce qu'**une dispersion d'encollage est utilisée, dans laquelle la quantité de polymère colloïdal est dans une gamme d'environ 150 à 250% en poids de l'agent d'encollage hydrophobe.

3. Procédé selon la revendication 1,
**caractérisé en ce qu'**une dispersion d'encollage est utilisée, qui contient au moins un agent d'encollage supplémentaire choisi dans le groupe constitué par l'anhydride succinique alcénylé et la colophane.

4. Procédé selon l'une quelconque des revendications 1 à 3, **caractérisé en ce que** ledit polymère colloïdal hydrosoluble est choisi dans le groupe de composés comprenant : les amidons, la carboxyméthylcellulose, l'éthylcellulose, les polyacrylamides, les polyéthylèneimines, les polyesters, les polyéthers, les polyamides, les poly(alcool vinylique), la gélatine, le tristéarate, la gomme arabique, les sucres ou leurs mélanges.

5. Procédé selon la revendication 4,
**caractérisé en ce que** ledit polymère colloïdal hydrosoluble est un amidon amphotère à faible viscosité.

6. Procédé selon la revendication 3,
**caractérisé en ce que** le composant d'encollage supplémentaire est un anhydride succinique alcénylé, dans une quantité de 20 à 70%, de manière avantageuse de 30 à 50%, en poids du dimère de cétène.

7. Procédé selon la revendication 3,
**caractérisé en ce que** le composant d'encollage supplémentaire est la colophane renforcée.

8. Procédé selon la revendication 3 ou 7, **caractérisé en ce que** le composant d'encollage supplémentaire est la colophane, dans une quantité d'environ 20 à 50% en poids du composé dimère de cétène.

9. Procédé selon l'une quelconque des revendications 1 à 8, **caractérisé en ce que** la dispersion d'encollage contient en outre un composé tensio-actif, un agent biocide et/ou un régulateur de pH.

10. Procédé selon la revendication 7 ou 8, **caractérisé en ce que** la dispersion d'encollage contient du sulfate d'aluminium, dans une quantité de 2 à 15% en poids dudit polymère colloïdal.

11. Procédé selon l'une quelconque des revendications 1 à 10, **caractérisé en ce que** ledit composé dimère de cétène est choisi dans le groupe constitué par les dimères de cétène alkylés, alcénylés, arylés et alkarylés.

12. Procédé selon l'une quelconque des revendications 1 à 11, **caractérisé en ce que** la teneur dudit agent d'encollage hydrophobe dans la dispersion d'encollage est d'environ 1 à 15% en poids, de manière avantageuse de 6 à 15% en poids.
